

## UNITED STATES PATENT OFFICE

1,948,276

PROCESS FOR INCREASING TENSILE  
STRENGTH OF CELLULOSE AND PROD-  
UCTAugust J. Pacini, Chicago, Ill., assignor to  
Milprint Products Corporation, Milwaukee,  
Wis., a corporation of WisconsinNo Drawing. Application May 4, 1931  
Serial No. 535,086

5 Claims. (Cl. 8—20)

My invention relates to a process for improvement in the properties, particularly the tensile strength, of cellulose materials, such as cotton, and to the product resulting from said process.

5 My invention consists in subjecting cellulose or textiles of cellulose materials to artificially produced ultra-violet radiation under controlled conditions effective to render the fibres of cellulose of greater tensile strength than they possess without this treatment.

10 It is commonly accepted that cellulose or textiles of cellulose are subject to deterioration, usually manifested as a loss in tensile strength, by the action of natural agents such as sunlight, and that the ultra-violet component of sunlight is charged with the greatest disintegrating effect (Johnson Textile Fabrics—page 309; Journal Society of Dyers and Colourists, Vol. 33, 1917, page 17; and Der Textilberichte 1924, page 745).

15 20 Ultra-violet radiation is charged with the development or formation of oxy cellulose which is a compound similar to that produced by overbleaching and which, by reason of its structureless, brittle or friable properties, is lacking in strength and hence reduces the tensile strength of the cellulose.

25 In accordance with this invention, however, cellulose is not only not weakened, but materially increased in tensile strength by subjection to, or treatment by, ultra-violet radiation under controlled conditions. This increase in the tensile strength properties is accomplished by exposure of the fibres or fabric to intense ultra-violet radiation of proper quantity and quality for a period

30 prior to the detectable formation of oxy cellulose.

35 If the treatment is prolonged until oxy cellulose is detectable, the process of deterioration sets in and the cellulose fibres are weakened instead of being strengthened. With a 110-volt quartz mercury vapor lamp, operating at maximum intensity, about 70 volts, and suspended substantially six inches from the fibres or fabric, the period of exposure has been found to materially increase tensile strength through a range of from eight-

40 tenths of a second to four and one-half seconds. The period during which oxy cellulose does not form, or at least is not detectable, may extend as long as fifteen or twenty minutes, depending upon such factors as the texture and number of fibres,

45 the relative surface exposed and the intensity and quality of ultra-violet radiation, but as the length of time of exposure approaches the point of formation of detectable oxy cellulose, the degree of increase in tensile strength becomes less.

50 Therefore, during this period prior to the forma-

tion of detectable oxy cellulose, the maximum increase in tensile strength of the cellulose determines the point at which to stop the treatment. As an instance of the efficacy of this method of increasing tensile strength of cellulose, cotton 60 fibres which have been given treatment equivalent to that which they would receive as fabric in the usual laundering process, have been increased in tensile strength as much at 21.21% when exposed for a period of eight-tenths of a second to the 65 ultra-violet radiation from a 110-volt quartz mercury arc lamp at six inches distance from the material.

During this period prior to the formation of oxy cellulose detectable by the known methods 70 of detection, a change in the cellulose takes place which increases the tensile strength very materially. I do not rest my invention upon any theory as to what the character of the change is, but tests indicate that by virtue of the ultra-violet radiation the alkali soluble component of 75 cellulose, generally designated beta-cellulose, is decreased by conversion into the alpha-cellulose component which has the property of greater tensile strength, and the additional alpha-cellulose formed by this conversion contributes to the 80 total strength of the fibre.

This treatment of cellulose can be applied after the cellulose is prepared into commercial fibres, such as thread or cord, or woven into fabrics, and, 85 because of the fact that the exposure to ultra-violet is relatively brief, the process does not slow down or otherwise affect the production of commercial material.

85 My invention is also applicable, for instance, 90 to the treatment of clothes in process of being laundered in commercial laundries, for the reason that the factors in the process can be arranged to conform to standard laundry practice with respect to the speed at which clothes are handled 95 in any of the steps or stages in the laundry operations.

I claim:

1. The process of imparting the property of 100 increased tensile strength to cellulose, which consists in subjecting cellulose to the action of artificially produced ultra-violet radiation and controlling the action thereof to prevent the formation of detectable oxy cellulose in said cellulose.

2. The process of imparting the property of 105 increased tensile strength to cellulose, which consists in subjecting the cellulose to the action of artificially produced ultra-violet radiation of given volume and intensity for a period of time and 110

stopping said action prior to the formation of detectable oxycellulose.

3. The herein described process which consists in strengthening cellulose fibre by exposing the cellulose to the action of ultra-violet radiation of given volume and intensity produced by a mercury vapor arc in quartz at a distance of substantially six inches from said arc and controlling the time of exposure to avoid the formation of detectable oxycellulose in said cellulose.
4. The herein described process which consists in strengthening cellulose fibre by exposing the cellulose for a period of time not in excess of fifteen minutes to the action of ultra-violet radiation such as produced by a mercury vapor

arc in quartz at a distance of substantially six inches from said arc, and of such volume and intensity as will not, during said period of exposure, form detectable oxycellulose.

5. The herein described process which consists in strengthening cellulose fibre by exposing the cellulose to the action of ultra-violet radiation such as produced by a mercury vapor arc in quartz at a distance of substantially six inches from said arc for substantially eight-tenths of a second, and of such volume and intensity as will not form detectable oxycellulose during said period of exposure.

AUGUST J. PACINI.

80

85

90

95

20

25

100

30

105

35

110

40

115

45

120

50

125

55

130

60

135

65

140

70

145

75

150